

## 1

**3,254,011**  
**ELECTROLYTIC POTASSIUM HYDROXIDE**  
**DESCALING**

Donald R. Zaremski, Cheswick, Pa., assignor to Allegheny Ludlum Steel Corporation, Brackenridge, Pa., a corporation of Pennsylvania  
 No Drawing. Filed Sept. 20, 1963, Ser. No. 310,504  
 8 Claims. (Cl. 204—140.5)

This application is a continuation-in-part of application Serial No. 42,964 dated July 15, 1960 entitled: "Caustic Bath," now Patent No. 3,121,026.

This invention relates to the removal of oxide scale from metals, and more particularly to an improved method for loosening and removing oxide scale from stainless steel strip.

During the processing of stainless steel from an ingot to a finished strip product, the in-process material is frequently heated in oxidizing atmospheres to temperatures at which oxide scale readily forms on the surface. This oxide scale is normally removed by conventional pickling baths, the steel strip being fed through the baths at a slow enough rate to effect removal of the oxide scale. However, when the scale-removing baths are used in conjunction with continuous annealing processes or the like, the scale-removing bath must be of sufficient strength to remove the scale as rapidly as the strip emerges from the furnace. In light gauge strip this speed may be rather rapid and since the speed of the strip is a critical factor in continuous annealing, this speed cannot be changed to accommodate the scale removal equipment. Because of this speed limitation and the tenacious nature of the scale of many types of stainless steel, special salt baths are required to loosen the scale and aid in its removal. These salt baths conventionally take the form of fused alkali metal hydroxides operating at temperatures from 800° F. to 1000° F. which tend to loosen the scale after which the strip is passed successively first into a bath of dilute sulfuric acid and then into a bath of mixed hydrofluoric and nitric acids. Although the high temperature salt baths are effective to loosen oxide scale, they tend to chemically attack the strip; they also have the additional disadvantages of attacking the various components of equipment required to retain the salt and guide the strip through the bath, such as tank linings, rolls, etc., which, in turn, can cause warping and distortion of lighter gauge strip.

In the parent application referred to above, an aqueous solution of potassium hydroxide operating at a relatively low temperature of about 400° F. is disclosed as having excellent properties in loosening and removing scale on titanium alloys and on stainless steel when used in place of the high temperature salt baths. This aqueous potassium hydroxide bath works excellently on titanium alloys and on some types of stainless steel; however, on certain types of stainless steel which form a very tenacious scale such as AISI Types 309, 310, 316 and 347, even this salt bath has proved to be too slow and inefficient for commercial application.

It is, accordingly, a principal object of this invention to provide an improved process for loosening and removing oxide scale from metal.

A more specific object of this invention is the provision of an improved salt bath-electrolytic treatment for loosening and removing scale from stainless steel.

Yet another object of this invention is to provide an improved process for continuously loosening and remov-

## 2

ing oxide scale from strip material, the process being adapted to be incorporated at the exit end of a continuous annealing line.

Still a further object of this invention is the provision of a relatively low temperature aqueous salt bath-electrolytic treatment to loosen and remove oxide scale from stainless steel having tenacious tightly-adhering oxide coatings.

Still a further, more general object of this invention is to provide a process for removing oxide scale from stainless steel strip, which process is also adapted to electro-polish the strip to a bright finish.

Still another more general object of this invention is the provision of an improved descaling bath for stainless steel.

These and other objects will become apparent from the following description taken in conjunction with the appended claims.

According to this invention, an aqueous solution of potassium hydroxide or an aqueous solution of potassium hydroxide and potassium nitrate is used as a descaling bath and electric current is passed through the bath and the stainless steel or other metal being descaled to effect descaling. (Potassium nitrate, if present, tends to increase the electropolishing capability of the bath as will be discussed presently, and has little effect on the scale removal characteristics. In any event, the term potassium hydroxide bath as used herein is intended to include baths having potassium nitrate as well as baths free of potassium nitrate.) It has been found that the use of electric current in conjunction with an aqueous potassium hydroxide bath substantially improves descaling results over the results from similar baths wherein no electric current is used with the scale from even the most difficult grades being removed quickly and completely. This improved result is readily apparent from a comparison of Tables I and II below, Table I showing the descaling results of an aqueous potassium hydroxide bath wherein no electric current was used and Table II showing the results of a similar aqueous potassium hydroxide bath wherein various current densities were passed through the bath and the steel. These Tables show results of controlled laboratory experiments for removing scale from small size samples of various types of stainless steel with various types of oxide scale.

TABLE I.—NON-ELECTROLYTIC AQUEOUS KOH DESCALING

| Alloy (AISI Grade) | Type Scale                | KOH Treatment <sup>1</sup> | Descaling Results  |
|--------------------|---------------------------|----------------------------|--------------------|
| 50                 | Finish Anneal             | ½, 1 and 2 min.            | Complete at 2 min. |
|                    | do                        | ½, 1 and 2 min.            | Complete at 1 min. |
|                    | do                        | 1 and 2 min.               | Do.                |
|                    | do                        | 2 min.                     | Complete.          |
|                    | do                        | 2 min.                     | Incomplete.        |
|                    | Intermediate Anneal       | 2 min.                     | Do.                |
| 55                 | Finish Anneal             | 2 min.                     | Do.                |
|                    | Intermediate Anneal       | 2 min.                     | Do.                |
|                    | Finish Anneal             | 2 min.                     | Do.                |
|                    | do                        | 2 min.                     | Do.                |
|                    | do                        | 1 and 2 min.               | Complete at 2 min. |
|                    | do                        | 1 and 2 min.               | Complete at 1 min. |
| 60                 | do                        | 2 min.                     | Complete.          |
|                    | do                        | 2 min.                     | Incomplete.        |
|                    | Intermediate Anneal       | 2 min.                     | Do.                |
|                    | Hot Roll-Normalize Anneal | 2 min.                     | Do.                |

<sup>1</sup> Caustic treatment in an aqueous solution of 80% KOH, 10%  $KNO_3$  and 10%  $H_2O$  maintained at about 425° F. followed by a 2 minute immersion in 15 percent  $H_2SO_4$  water solution at 150° F., and a 2 minute immersion in 10 percent  $HNO_3$ -2 percent HF water solution at 125° F.

TABLE II.—(ELECTROLYTIC) AQUEOUS KOH DESCALING

| Alloy<br>(AISI<br>Grade) | Type Scale                         | Time,<br>min. | KOH<br>Treatment <sup>1</sup><br>Anodic<br>Current<br>Density,<br>amp./in. <sup>2</sup> | Descaling Results               |
|--------------------------|------------------------------------|---------------|-----------------------------------------------------------------------------------------|---------------------------------|
| 201                      | Finish Anneal                      | 1             | 0.125                                                                                   | Complete.                       |
| 301                      | do                                 | 1             | 0.125                                                                                   | Do.                             |
| 304                      | do                                 | 1             | 0.125                                                                                   | Do.                             |
| 310                      | do                                 | 1.5           | 0.250                                                                                   | Do.                             |
| 310                      | Intermediate Anneal                | 1.5           | 0.350                                                                                   | Do.                             |
| 316                      | Finish Anneal                      | 1.5           | 0.250                                                                                   | Do.                             |
| 316                      | Intermediate Anneal                | 1.5           | 0.350                                                                                   | Do.                             |
| 316                      | do                                 | 2             | 0.750                                                                                   | Complete plus polished surface. |
| 321                      | Finish Anneal                      | 1.5           | 0.250                                                                                   | Complete.                       |
| 347                      | do                                 | 1.5           | 0.250                                                                                   | Do.                             |
| 410                      | do                                 | 1             | 0.250                                                                                   | Do.                             |
| 430                      | do                                 | 1             | 0.125                                                                                   | Do.                             |
| 430                      | Intermediate Anneal                | 1.5           | 0.350                                                                                   | Complete plus bright surface.   |
| 430                      | do                                 | 2             | 1.000                                                                                   | Complete plus polished surface. |
| 430                      | Hot Roll-Normalize-<br>Box Anneal. | 2             | 0.350                                                                                   | Incomplete.                     |
| 430                      | do                                 | 5             | 1.000                                                                                   | Complete.                       |

<sup>1</sup> Caustic treatment in an aqueous solution of 80% KOH, 10% KNO<sub>3</sub> and 10% H<sub>2</sub>O maintained at about 425° F., followed by 1 minute immersion in 10 percent H<sub>2</sub>SO<sub>4</sub> at 125° F.

From Table I it can be readily seen that with an aqueous potassium hydroxide bath satisfactory descaling results are obtained on stainless steel having scale that is relatively easily removed, such as AISI Types 201, 301, 302, 304 and 410, and certain types of scale on Type 430 without the use of electric current. However, on the material have scale which is difficult to remove, such as Types 309, 310, 316, 321 and 347 and some types of scale on Type 430, the results listed in Table I clearly show that the use of an aqueous potassium hydroxide bath without electric current will not completely remove the scale in two minutes. Because of the required use of descaling in conjunction with other processes such as continuous annealing, a time requirement of greater than

25 positive electrodes (anodes), and thence into the second compartment in which were disposed negative electrodes (cathodes). This bi-polar type of bath was used to insure consistent results in preference to a single bath having a positive roll contacting the strip and negative grids in the bath. With the contacting roll maintaining the strip positive throughout the bath better scale removal results, but arcing at the roll may be a problem with smaller diameter rolls and heavier gauge strip, especially at higher current densities, hence, the preference for the bi-polar bath. The current densities were varied as shown in 30 Table III, producing the results indicated therein. Two tanks A and B following the potassium hydroxide bath 35 were filled with acid as indicated.

TABLE III.—CONTINUOUS AQUEOUS KOH DESCALING OF TYPE 316 STAINLESS STEEL

| Caustic Treatment <sup>1</sup>             | Acid Treatment                                                                 |                                                                  | Speed,<br>f.p.m. | Results and Comments                              |
|--------------------------------------------|--------------------------------------------------------------------------------|------------------------------------------------------------------|------------------|---------------------------------------------------|
|                                            | Tub A                                                                          | Tub B                                                            |                  |                                                   |
| Non-Electrolytic                           | 15% H <sub>2</sub> SO <sub>4</sub> at 140° F.                                  | 7% HNO <sub>3</sub> —2% HF at 100° F.                            | 2                | No descaling.                                     |
| Do                                         | 15% H <sub>2</sub> SO <sub>4</sub> at 140° F. and 0.5<br>amp./in. <sup>2</sup> | do                                                               | 2                | Do.                                               |
| Do                                         | 5% H <sub>2</sub> SO <sub>4</sub> at 130° F. and 1.0<br>amp./in. <sup>2</sup>  | 7% HNO <sub>3</sub> —2% HF at 98° F.                             | 2                | Do.                                               |
| Do                                         | 5% H <sub>2</sub> SO <sub>4</sub> at 140° F. and 0.5<br>amp./in. <sup>2</sup>  | 10% HNO <sub>3</sub> at 130° F. and 0.5<br>amp./in. <sup>2</sup> | 1.3              | Do.                                               |
| Electrolytic at 0.25 amp./in. <sup>2</sup> | 5% H <sub>2</sub> SO <sub>4</sub> at 95° F. and 0.25<br>amp./in. <sup>2</sup>  | 7% HNO <sub>3</sub> —2% HF at 125° F.                            | 1.3              | Descaling complete.                               |
| Do                                         | do                                                                             | No acid                                                          | 1.3              | Do.                                               |
| Do                                         | 5% H <sub>2</sub> SO <sub>4</sub> at 95° F.                                    | 7% HNO <sub>3</sub> —2% HF at 125° F.                            | 1.3              | Do.                                               |
| Do                                         | do                                                                             | No acid                                                          | 1.3              | Do.                                               |
| Do                                         | do                                                                             | do                                                               | 2                | Do.                                               |
| Do                                         | do                                                                             | do                                                               | 3                | Do.                                               |
| Electrolytic at 2 amp./in. <sup>2</sup>    | do                                                                             | do                                                               | 1.3              | Descaling complete with<br>surface electropolish. |

<sup>1</sup> Aqueous solution of 80% KOH, 10% KNO<sub>3</sub> and 10% H<sub>2</sub>O maintained at about 425° F.

two minutes tends to negative the commercial practicability of the process. The data in Table II shows when electric current is used in conjunction with the aqueous potassium hydroxide-potassium nitrate bath, the scale is easily removed even on most of these "difficult" grades within the two-minute requirement and, hence, is applicable for commercial production.

In order to establish the commercial feasibility of this process, several strips of AISI Type 316 stainless steel (a "difficult" grade) having oxide coatings, were passed continuously through an aqueous solution of potassium hydroxide at various speeds with varied amounts of electric current being used and several different acid dips being given following the potassium hydroxide treatment. The electric current was applied by means of a bi-polar system in which the tank of aqueous potassium hydroxide was divided into two compartments. The strip passed into the first compartment in which were disposed posi-

60 The results listed in Table III clearly show the superiority of the electrolytic potassium hydroxide treatment over a similar non-electrolytic treatment applied to a strip continuously drawn through the bath. The data from this table show that electrolytic treatment is sufficiently rapid for use commercially in connection with a continuous annealing furnace and will completely 65 descale even "difficult" alloys at the required rapid line speeds. Also, from an examination of Tables II and III, it can be seen that the conventional dual acid treatment following the potassium hydroxide treatment can be eliminated and a single treatment in aqueous 5% sulfuric acid is sufficient to remove the stain from the surface of the strip. Further, there is no need for passing any current through the sulfuric acid bath as has been the prior art practice. Table IV below shows the descaling results of various concentrations of potassium hydroxide 70 and potassium hydroxide-potassium nitrate baths on de-

scaling of Type 316 stainless steel and also shown for comparison are sodium hydroxide and sodium hydroxide-sodium nitrate baths.

but also will be oxidized to a form which will readily separate from the surface of the strip and enter the potassium hydroxide bath. But, in the two-tank set-up described,

TABLE IV.—KOH VS. NaOH DESCALING BATH EVALUATION  
[Type 316 Stainless Steel<sup>1</sup>]

| Percent<br>Caustic | Percent<br>Nitrate   | Percent<br>H <sub>2</sub> O | Temp.,<br>° F. | .25 amp./in. <sup>2</sup>   |                              | .50 amp./in. <sup>2</sup>   |                              | 1.0 amp./in. <sup>2</sup>   |                              | 2.0 amp./in. <sup>2</sup>   |                              | 3.0 amp./in. <sup>2</sup>   |                              |
|--------------------|----------------------|-----------------------------|----------------|-----------------------------|------------------------------|-----------------------------|------------------------------|-----------------------------|------------------------------|-----------------------------|------------------------------|-----------------------------|------------------------------|
|                    |                      |                             |                | Percent<br>scale<br>removal | Bright-<br>ness <sup>2</sup> | Percent<br>scale<br>removal | Bright-<br>ness <sup>2</sup> | Percent<br>scale<br>removal | Bright-<br>ness <sup>2</sup> | Percent<br>scale<br>removal | Bright-<br>ness <sup>2</sup> | Percent<br>scale<br>removal | Bright-<br>ness <sup>2</sup> |
| 90 KOH             |                      | 10                          | 400            | 100                         | 22                           | 100                         | 24                           | 100                         | 20                           | 100                         | 32                           | 100                         | 36                           |
| 80 KOH             |                      | 20                          | 400            | 100                         | 18                           | 100                         | 20                           | 100                         | 12                           | 100                         | 16                           | 100                         | 18                           |
| 70 KOH             |                      | 30                          | 400            | 90                          | 6                            | 90                          | 7                            | 80                          | 7                            | 85                          | 6                            | 90                          | 7                            |
| 60 KOH             |                      | 40                          | 315            | 80                          | 5                            | 85                          | 6                            | 85                          | 6                            | 85                          | 6                            | 85                          | 5                            |
| 50 KOH             |                      | 50                          | 250            | 90                          | 6                            | 90                          | 6                            | 85                          | 6                            | 80                          | 4                            | 75                          | 4                            |
| 40 KOH             |                      | 60                          | 250            | 90                          | 7                            | 90                          | 7                            | 90                          | 6                            | 90                          | 7                            | 90                          | 7                            |
| 30 KOH             |                      | 70                          | 230            | 85                          | 7                            | 85                          | 6                            | 85                          | 6                            | 80                          | 7                            | 80                          | 6                            |
| 25 KOH             |                      | 75                          | 220            | 50                          | 3                            | 50                          | 2                            | 50                          | 2                            | 50                          | 3                            | 50                          | 3                            |
| 90 KOH             | 5 KNO <sub>3</sub>   | 5                           | 400            | 100                         | 23                           | 100                         | 18                           | 100                         | 32                           | 100                         | 29                           | 100                         | 33                           |
| 80 KOH             | 10 KNO <sub>3</sub>  | 10                          | 400            | 100                         | 20                           | 100                         | 13                           | 100                         | 30                           | 100                         | 30                           | 100                         | 32                           |
| 70 KOH             | 20 KNO <sub>3</sub>  | 10                          | 400            | 100                         | 15                           | 100                         | 12                           | 100                         | 17                           | 100                         | 16                           | 100                         | 22                           |
| 60 KOH             | 30 KNO <sub>3</sub>  | 10                          | 400            | 100                         | 12                           | 100                         | 9                            | 100                         | 6                            | 100                         | 4                            | 100                         | 4                            |
| 70 KOH             | 10 KNO <sub>3</sub>  | 20                          | 400            | 85                          | 8                            | 85                          | 6                            | 85                          | 5                            | 85                          | 6                            | 90                          | 7                            |
| 60 KOH             | 20 KNO <sub>3</sub>  | 20                          | 400            | 80                          | 3                            | 85                          | 5                            | 85                          | 6                            | 85                          | 5                            | 80                          | 4                            |
| 50 KOH             | 40 KNO <sub>3</sub>  | 10                          | 400            | 90                          | 7                            | 90                          | 8                            | 90                          | 7                            | 100                         | 7                            | 100                         | 6                            |
| 50 KOH             | 20 KNO <sub>3</sub>  | 30                          | 365            | 80                          | 5                            | 80                          | 5                            | 80                          | 5                            | 80                          | 4                            | 85                          | 4                            |
| 25 KOH             | 25 KNO <sub>3</sub>  | 50                          | 240            | 80                          | 5                            | 80                          | 5                            | 80                          | 5                            | 85                          | 5                            | 80                          | 5                            |
| 90 NaOH            |                      | 10                          | (3)            |                             |                              |                             |                              |                             |                              |                             |                              |                             |                              |
| 80 NaOH            |                      | 20                          | 400            |                             |                              |                             |                              |                             |                              |                             |                              |                             |                              |
| 70 NaOH            |                      | 30                          | 350            | 75                          | 4                            | 75                          | 4                            | 75                          | 3                            | 70                          | 3                            | 70                          | 3                            |
| 60 NaOH            |                      | 40                          | 325            | 80                          | 5                            | 80                          | 5                            | 80                          | 6                            | 75                          | 5                            | 75                          | 3                            |
| 50 NaOH            |                      | 50                          | 285            | 80                          | 4                            | 85                          | 7                            | 80                          | 5                            | 75                          | 4                            | 75                          | 5                            |
| 90 NaOH            | 5 NaNO <sub>3</sub>  | 5                           | (4)            |                             |                              |                             |                              |                             |                              |                             |                              |                             |                              |
| 80 NaOH            | 10 NaNO <sub>2</sub> | 10                          | (4)            |                             |                              |                             |                              |                             |                              |                             |                              |                             |                              |
| 70 NaOH            | 20 NaNO <sub>2</sub> | 10                          | (4)            |                             |                              |                             |                              |                             |                              |                             |                              |                             |                              |
| 60 NaOH            | 20 NaNO <sub>2</sub> | 20                          | 400            | 90                          | 5                            | 95                          | 5                            | 95                          | 5                            | 90                          | 5                            | 90                          | 5                            |
| 50 NaOH            | 20 NaNO <sub>2</sub> | 30                          | 330            | 90                          | 6                            | 90                          | 6                            | 85                          | 4                            | 85                          | 5                            | 90                          | 6                            |
| 25 NaOH            | 25 NaNO <sub>2</sub> | 50                          | 245            | 90                          | 7                            | 95                          | 6                            | 90                          | 5                            | 85                          | 5                            | 85                          | 5                            |

<sup>1</sup> Each sample was given a two minute treatment in the bath indicated at the temperature and current density indicated and then rinsed in a 5% aqueous solution of sulfuric acid.

<sup>2</sup> Surface reflectivity readings as measured by gloss meter sensing head, Model No. 660M and recording unit, Model No. 610 manufactured by Photovolt Corporation, New York, New York.

<sup>3</sup> Could not get NaOH into solution at operating temperature or above.

<sup>4</sup> Could not get NaOH and NaNO<sub>3</sub> into solution at operating temperature or above.

From Table IV above, it can be seen that in order to achieve 100% descaling in two minutes, which for commercial reasons is the longest permissible time, an aqueous potassium hydroxide bath free of nitrate additions must have at least an 80% concentration of potassium hydroxide and when potassium nitrate is present in the bath, there must be at least 60% potassium hydroxide present and the combined percentage of potassium hydroxide and potassium nitrate must be at least 90%. It can also be seen from Table IV that aqueous sodium hydroxide baths and sodium hydroxide-sodium nitrate baths are not effective in any concentration to remove 100% of the scale in two minutes. Another benefit that can be derived from the electrolytic descaling in the baths of this invention is an electropolishing of the surface of the steel in addition to scale removal. This can be seen from Table IV in which gloss readings as high as 36 are produced on the stainless steel. This is a substantial amount of polishing since the original surface gloss of the material before scaling was less than about 10. It should be noted that no appreciable amount of electropolishing occurs when the potassium hydroxide content is below 70% such as when there is 60% potassium hydroxide and 30% potassium nitrate, and even at 70% potassium hydroxide and 20% potassium nitrate, the surface gloss is not raised to above 20 until the current density is at least 3 amps. per square inch.

It has been found that there must be at least 5% water in the bath for the bath to be suitably electrically conducting. Also, the temperature of the bath should not exceed about 500° F. or the water will be driven off and the bath will become anhydrous and unsuitable for the practice of this invention.

It is preferred, in the practice of this invention, that the strip be anodic or positive during at least a portion of the treatment so that the scale will not only be loosened

40 the strip must be cathodic during at least a portion of the process. This portion when the strip is cathodic should be kept to a minimum since it is not as effective for scale removal and since electropolishing will not occur when the strip is cathodic. With the two compartment arrangement of the tank as described above, the strip is maintained cathodic in the first compartment and anodic in the second.

Although several embodiments of this invention have been shown and described, various adaptations and modifications may be made without departing from the scope and appended claims.

I claim:

1. In a process for removing oxide scale from stainless steel the improvement which comprises, immersing said steel in an aqueous bath having at least 80% potassium hydroxide and no less than 5% water, maintaining said bath at a temperature of less than 500° F., and passing an electric current through said bath and said steel.
2. The process of claim 1 wherein the current density is maintained at a value of at least .125 ampere per square inch of steel surface immersed in the bath.
3. The process of claim 2 wherein the steel is immersed in a second bath of dilute acid after scale removal.
4. The process of claim 2 wherein at least a portion of the strip in the bath is maintained anodic whereby to electropolish the strip.
5. In a process for removing oxide scale from stainless steel the improvement which comprises, immersing said steel in an aqueous bath having at least 60% potassium hydroxide, and from 5% to 30% potassium nitrate and wherein the total amount of potassium hydroxide and potassium nitrate is from 90% to 95%, maintaining said bath at a temperature of less than 500° F., and passing an electric current through said bath and said steel.

6. The process of claim 5 wherein the current density is maintained at a value of at least .125 ampere per square inch of steel surface immersed in the bath.

7. The process of claim 6 wherein the steel is immersed in a second bath of dilute acid after scale removal.

8. The process of claim 6 wherein at least a portion of the strip in the bath is maintained anodic whereby to electropolish the strip.

## References Cited by the Examiner

## UNITED STATES PATENTS

|             |        |               |         |
|-------------|--------|---------------|---------|
| 2,797,193   | 7/1957 | Eigler et al. | 204—143 |
| 3,096,261   | 7/1963 | Mekjean       | 204—145 |
| 5 3,121,026 | 2/1964 | Beigay        | 134—2   |

JOHN H. MACK, Primary Examiner.

R. HARDER, R. MIHALEK, Assistant Examiners.